

## UNITED STATES PATENT OFFICE

2,172,475

PROCESS FOR THE ENNOBLEMENT OF TEX-  
TILE MATERIALS AND PRODUCTS THERE-  
FROMWalther Kaase and Ernst Waltmann, Krefeld,  
Germany, assignors to Heberlein Patent Cor-  
poration, New York, N. Y., a corporation of  
New YorkNo Drawing. Application February 29, 1936, Se-  
rial No. 66,498. Renewed October 6, 1938. In  
Germany March 1, 1935

## 8 Claims. (Cl. 8—120)

This invention relates to increasing water-repellence in textile materials and particularly cellulose-containing materials; and to products obtained thereby.

5 In the ennobling of such textiles in the past in order to make them resistant to water there has been suggested a number of processes which are based mainly on the surface treatment of the said materials with esterifying agents such as fatty acid chlorides or fatty acid anhydrides. In the carrying out of these prior processes on a large scale considerable difficulties have been encountered due on the one hand to unfavorable reaction conditions whereby the appearance and feel of the goods is changed, and on the other hand because these processes require considerable time in operation as well as the expenditure of considerable money for materials.

10 The principal object of the present invention is to ennable cellulose-containing materials such as cotton, jute, linen, hemp and rayon made of cellulose or derivatives of the same to render them resistant to water, by a simple process which may be carried out in a relatively short time and less expensively than heretofore; and to produce products having improved characteristics thereby.

15 The invention accordingly comprises the novel products as well as the novel processes and steps of processes according to which such products are manufactured, the specific embodiments of which are described hereinafter by way of example and in accordance with which we now prefer to practice the invention.

20 It has now been found that the ennobling of these textiles can be effected within a very short period of time while at the same time giving the desired protection to the fibrous material if one subjects the textile materials to asymmetric fatty acid anhydrides, which may also be spoken of as asymmetric di-acyl oxides.

25 By the expression asymmetric fatty acid anhydrides there shall be understood those anhydrides which contain one acyl residue of at least 10 carbon atoms while the other acyl residue contains not more than 4 carbon atoms and preferably 2 carbon atoms. The principle involved in employing materials of this type for the treatment of these cellulose-containing materials is that these asymmetric anhydrides break up on heating so that from two mols of asymmetric anhydride there is split off one mol of the acyl radical having the low number of carbon atoms (for example this might be acetic acid) and this split-off acid volatilizes. Thereupon there is pro-

duced on the fiber in the nascent state a fatty acid anhydride containing at least 10 carbon atoms and this fatty acid anhydride in the nascent state reacts with exceptional ease with the cellulose to cause esterification which is usually 5 a superficial one sufficient to give the water-repellence desired.

These asymmetric fatty acid anhydrides may be obtained in an extremely simple and satisfactory manner on an industrial scale by the reaction of ketenes containing not more than 4 carbon atoms on fatty acids containing at least 10 carbon atoms.

10 In the place of the common fatty acids there may be employed with similar success fatty acids, the carbon chain of which is interrupted by atoms or atomic groups S, O, CO, O.CO, NR, NR.CO, CO.NR, SO<sub>2</sub>, NR.SO<sub>2</sub>, SO<sub>2</sub>.NR, in which R may represent hydrogen or any desired hydrocarbon residue. These compounds are covered 15 herein by the expression—asymmetric fatty acid anhydrides—as defined above.

15 As examples of useful products corresponding to the substances mentioned are the reaction of ketenes on lauric acid, palmitic acid, myristic acid, stearic acid, technical stearine, hydrogenated-fish-oil-fatty acid, the adipic-acid ester of octadecylalcohols, the palmitic ether of glycolic acid, the myristyl ether of thio-glycolic acid, the stearic acid ester of glycolic acid, the monooctyl 20 ester of di-glycolic acid, N-didodecylamino acetic acid, cetyl-amide of sulfo-acetic acid, stearylamino acetic acid; to form the corresponding asymmetric fatty acid anhydrides of the ketenes selected with the substances just listed. The ketenes 25 are selected to give an acyl residue of 4 carbon atoms or less.

25 The new substances have great reactivity with respect to such textile materials, especially the cellulose and cellulose derivatives hereinabove mentioned, so that the action thereon takes place within a very short time without the need for special auxiliary reagents. It is only necessary to expose the materials impregnated with the mixed anhydrides to certain temperatures with drying. First a preliminary drying at about 100° C. for evaporation of the solvent, if employed, occurs and subsequently a drying at an increased temperature of about 140–160° C. for the splitting off and expelling of the anhydrides having the lower number of carbon atoms.

30 The impregnation of the textile material with the products described may be effected in any desired manner with or without the use of organic solvents, by emulsifying an aqueous solu- 35

tion of the anhydride and then treating the textile by immersion, spraying or the like. A catalyst may be employed for obtaining the desired effect, but it is not necessary.

5 The following are examples of embodiments of the invention which are given only as illustrations of the invention:

*Examples*

10 1. A fabric of viscose warp and viscose crepe filling is passed through a 1% solution of asymmetric stearic acid-acetic acid anhydride in light benzene, suction filtered and thereupon exposed for 5 minutes to a temperature of 100° C. This is followed by a treatment at 150° C. for 5 minutes. The fabric thereupon has an excellent water-repellent property and its feel and the color have not been influenced in any manner whatsoever. This effect is also resistant to easy house laundering and is also not affected by treatments with organic solvents of the kind used by chemical cleaners.

15 2. A fabric of a warp of acetate silk and a filling of viscose crepe is sprayed with a 1% solution of adipic-acid-stearic alcohol ester-acetic acid anhydride in benzene and thereupon treated for 4 minutes at 100° C. This is followed by a treatment at 160° C. for 5 minutes. The fabric is thereupon water-repellent.

20 3. A fabric with a warp of acetate silk and a filling of viscose crepe is passed through a 1% solution of adipic-acid-stearic alcohol ester-acetic acid-anhydride in benzene, thereupon treated for 1 minute at 100° C. and subsequently for 5 minutes at 150° C. The fabric is thereupon water-repelling.

25 As an example of the reaction which occurs upon treating textile material such as cellulose-containing material with an asymmetric anhydride in accordance with our invention, whereby one component of the asymmetric anhydride is volatilized, we give the following reaction



30 It will be noticed in this reaction acetic acid is liberated and volatilizes on heating under suitable conditions to cause a superficial esterification of the cellulose by the remainder of the asymmetric anhydride.

35 In the claims where the expression "cellulose-containing material" is employed it is intended to cover fibers, yarns, fabrics or other forms of cotton, jute, linen, hemp and rayon including viscose, cuprammonium, or other precipitated cellulose or derivatives of cellulose such as acetyl cellulose.

40 While the invention has been described in detail according to the preferred manner of carrying out the process, it will be obvious to those skilled in the art after understanding the invention that changes and modifications may be made therein without departing from the spirit or scope of the invention, and it is intended in the appended claims to cover all such changes and modifications.

45 What is claimed as new and desired to be secured by Letters Patent is:

50 1. A process for the ennobling of textile ma-

5 terials which comprises applying to the textile material an asymmetric fatty acid anhydride containing a long acyl radical of at least 10 carbon atoms and a considerably shorter acyl radical capable of being split off upon heating, and heating to split off the shorter acyl radical and to cause a reaction of the textile material with the remainder of said anhydride.

55 2. A process for ennobling textile material which comprises applying to the textile material an asymmetric fatty acid anhydride having one acyl residue of at least 10 carbon atoms and another acyl residue containing not more than 4 carbon atoms, to increase the water-repellence and to decrease the tendency to spotting of said material and heating to split off the acyl residue of not more than four carbon atoms to cause reaction of the textile material with the remainder of said fatty acid anhydride.

60 3. A process for ennobling cellulose-containing material which comprises applying to the textile material an asymmetric fatty acid anhydride having one acyl residue of at least 10 carbon atoms and another acyl residue containing not more than 4 carbon atoms, to increase the water-repellence and to decrease tendency to spotting of said material and heating to about 100° C. or over to split off the acyl residue of not more than four carbon atoms to cause reaction of the textile material with the remainder of said fatty acid anhydride.

65 4. A process for ennobling cellulose-containing material which comprises treating cellulose-containing material with an asymmetric fatty acid anhydride having two acyl residues, having one acyl residue of at least 10 carbon atoms and the other acyl residue having not more than 4 carbon atoms, and heating the cellulose-containing material so treated to volatilize the acyl residue having the lower number of carbon atoms, to increase the water-repellence and to decrease tendency to spotting of said material.

70 5. A process according to claim 4 in which the anhydride is combined with the cellulose-containing material in the presence of a solvent and is thereafter heated first to remove the solvent and then to a higher temperature to break up the anhydride and cause partial esterification of the cellulose by the acyl residue containing at least 10 carbon atoms.

75 6. A process for ennobling cellulose-containing material which comprises subjecting artificial silk to the action of stearic acid-acetic acid anhydride, and thereafter heating the silk so treated to about 150° C. for about 5 minutes to produce a water-repellent property therein.

80 7. A process according to claim 6 in which adipic acid-stearic alcohol ester-acetic acid anhydride is substituted for the stearic acid-acetic acid anhydride, followed by a heating to about 160° C. for about 5 minutes.

85 8. A cellulose-containing textile product being superficially combined with a fatty acid radical having at least ten carbon atoms, said material having a water-repellent property which is fast to washing but in appearance and feel being substantially the same as the untreated textile product, said product being made according to the process of claim 1.

90 WALTHER KAASE.  
ERNST WALTMANN. 70

CERTIFICATE OF CORRECTION.

Patent No. 2,172,475.

September 12, 1939.

WALTHER KAASE, ET AL.

It is hereby certified that error appears in the printed specification of the above numbered patent requiring correction as follows: Page 2, second column, line 20, claim 3, for "cellulose-containing" read textile; and that the said Letters Patent should be read with this correction therein that the same may conform to the record of the case in the Patent Office.

Signed and sealed this 10th day of October, A. D. 1939.

(Seal)

Henry Van Arsdale,  
Acting Commissioner of Patents.